

L. S. HUGHES.

METHOD OF MAKING ZINC OXID.

APPLICATION FILED NOV. 13, 1906. RENEWED NOV. 27, 1908.

920,337.

Patented May 4, 1909.



WITNESSES:

John William  
Stewart

INVENTOR

BY

Louis S. Hughes

Francis J. Chambers,  
his ATTORNEY.

# UNITED STATES PATENT OFFICE.

LOUIS S. HUGHES, OF JOPLIN, MISSOURI, ASSIGNOR TO PICHER LEAD COMPANY, OF JOPLIN, MISSOURI, A CORPORATION OF MISSOURI.

## METHOD OF MAKING ZINC OXID.

No. 920,337.

Specification of Letters Patent.

Patented May 4, 1909.

Application filed November 13, 1906, Serial No. 343,284. Renewed November 27, 1908. Serial No. 464,785.

*To all whom it may concern:*

Be it known that I, LOUIS S. HUGHES, a citizen of the United States of America, residing in Joplin, in the county of Jasper and 5 State of Missouri, have invented a certain new and useful Improvement in Methods of Making Zinc Oxid, of which the following is a true and exact description, reference being had to the accompanying drawings, which 10 form a part thereof.

My invention relates to the manufacture of zinc oxide from zinc carbonate having special reference of course to the native carbonate ores. 15 The object of my invention is to provide for a rapid, efficient, and economical manufacture of zinc oxide from such ores my improved method, broadly speaking, consisting in finely dividing the carbonate, maintaining 20 the furnace at an internal temperature sufficient to decompose the carbonate with a production of zinc oxide  $ZnO$  and carbonic acid  $CO_2$ . I then inject the finely divided carbonate into the heat zone of the furnace 25 in a fine state of separation, as by means of a feed jet of air or vapor, a rapid decomposition of the ore taking place and zinc oxide in an exceedingly fine state of division passing out of the furnace with the gases is then 30 separated by screening, the separation of the heavy impurities being effected by subsidence either in the furnace or in the flues intervening between the furnace and the screen system, and for the best results my process 35 should be practiced in a vertical furnace, the air or vapor jet being directed upward from the bottom of the furnace and provision made for the extraction of heavy impurities from the bottom of the furnace.

It is an important feature of my invention that the furnace should be maintained 40 at temperatures not above  $1300^{\circ} F.$  for the reason that the body of the zinc oxide is impaired by temperatures materially in excess 45 of that amount and for the further reasons that a greater furnace heat develops a greater brilliancy of color in any iron oxid which may remain in admixture with the zinc oxide and the further reason that cadmium 50 which is very frequently found in zinc ores is not burned to an oxid at this temperature while at higher temperatures it is oxidized and forms a discoloring agent.

My process is most advantageously carried 55 into effect in furnaces of the character

described in my copending applications, one filed March 20, 1906 Serial Number 306,954 and the other filed October 22, 1906, Serial Number 339,894, and I have illustrated such a furnace in the drawings forming part of 60 this specification and in which—

Figure 1 is a side elevation of a furnace with connected flues and screen system, the furnace being partly shown in vertical section, and Fig. 2 is a cross-section on the line 65 2—2 of Fig. 1.

A indicates the cylindrical walls of the furnace formed of thin unlined sheet metal and provided with a hopper shaped bottom A' of the same material having one or more 70 openings indicated at A<sup>2</sup> for the admission of air and the outlet of unburned particles which settle in the furnace; A<sup>3</sup> indicating the normally closed opening by which access is had to the interior of the furnace. 75

D is an air jet pipe directed axially upward from the bottom of the furnace and supplied by an air pipe B'.

C is a flue leading from the top of the furnace provided with settling chambers C' C' 80 and connecting, as shown, to a draft fan D, with the flues C<sup>2</sup>, C<sup>3</sup>, the latter flue having hoppers C<sup>4</sup>, C<sup>4</sup>, opening into its bottom for the reception of the zinc oxide and connecting at top with screen bags indicated at E, 85 E, through which the furnace gases escape.

F indicates a gas pipe supplying an annular gas ring F' having projecting from it a series of burner nozzles F<sup>2</sup>, F<sup>3</sup>, these burner nozzles projecting into the burner 90 tubes G, G, which extend through the walls of the furnace and beyond the same, the inner ends of the burner tubes having overhangs, as indicated at G'.

G is a hopper in which the finely divided 95 ore is placed and which communicates with the interior of the furnace through a chute H' having a trough like end H<sup>2</sup> which projects to or nearly to the center of the furnace so as to deliver the ore directly into the 100 upwardly moving air jet from the jet pipe.

I is a gate for regulating the feed and J a rapping or vibrating device acting on the hopper and chute so as to keep the metal of which they are made in vibration and insure 105 a constant and even feed of ore.

In operation the furnace is heated by the admission of the mixed gas and air entering through the burner tubes G and forming a central core of flame, as indicated at K, sur- 110

rounded and jacketed, especially in the lower part of the furnace, by air indicated at L, this air entering through the opening A<sup>2</sup>. The finely divided zinc carbonate is placed in the hopper H and fed through the chute H' and trough H<sup>2</sup> to the center of the air jet issuing from the pipe B by which it is projected into the heat zone of the furnace in a fine state of separation as well as division. 10 The zinc carbonate is decomposed into zinc oxide and carbonic acid and the overheating of the zinc oxide prevented by the rapid eduction through the thin walls of the furnace of excessive heat so that the temperature of the furnace can be readily maintained not in excess of 1300° F. The heavier unburned particles of ore, cinder, etc., settle in the vertical furnace and finally escape through the opening A<sup>2</sup> while the zinc oxide and furnace gases escape through the flue C depositing the heavier impurities in the settling chamber C' and finally being separated from each other in the screen system E, the 15 oxide collecting in the hoppers C<sup>4</sup>. 20 25 Having now described my invention what I claim as new and desire to secure by Letters Patent is—

1. The method of manufacturing zinc oxide from zinc carbonate which consists in finely dividing the carbonate, maintaining a furnace at an internal temperature sufficient to decompose the carbonate by an internal gas flame, injecting the finely divided carbonate into the heated portion of the furnace by a jet of air or vapor directed upward from the bottom of the furnace to decompose it, and separating the zinc oxide and furnace gases from the gases by screening.

nace to decompose it, separating the zinc 55 oxide and furnace gases from impurities by subsidence and separating the zinc oxide from the gases by screening.

2. The method of manufacturing zinc oxide from zinc carbonate which consists in 40 finely dividing the carbonate, maintaining a furnace at an internal temperature sufficient to decompose the carbonate by an internal gas flame, injecting the finely divided carbonate into the heated portion of the furnace 45 by a jet of air or vapor directed upward from the bottom of the furnace to decompose it, and separating the zinc oxide and furnace gases from the gases by screening.

3. The method of manufacturing zinc 50 oxide from zinc carbonate which consists in finely dividing the carbonate, maintaining a furnace at an internal temperature sufficient to decompose the carbonate by an internal gas flame, cooling the furnace to maintain 55 its temperature below that at which the zinc oxide is impaired by heat and heat products, injecting the finely divided carbonate into the heated portion of the furnace to decompose it, separating the zinc oxide and furnace 60 gases from impurities by subsidence and separating the zinc oxide from the gases by screening.

LOUIS S. HUGHES.

Witnesses:

BELLE SPARKS,  
JERE. CHARLOW.